

(No Model.)

J. A. HUNTER.  
COMPOSITE STEEL PLATE.

No. 537,463.

Patented Apr. 16, 1895.

FIG. 1.



FIG. 2.



FIG. 3.



Witnesses:

J. D. Goodwin  
Frank C. Bechtold  


Inventor:

John A. Hunter  
by his Attorneys



# UNITED STATES PATENT OFFICE.

JOHN A. HUNTER, OF PHILADELPHIA, PENNSYLVANIA.

## COMPOSITE STEEL PLATE.

SPECIFICATION forming part of Letters Patent No. 537,463, dated April 16, 1895.

Application filed November 13, 1893. Serial No. 490,787. (No model.)

*To all whom it may concern:*

Be it known that I, JOHN A. HUNTER, a citizen of the United States, residing in Philadelphia, Pennsylvania, have invented certain 5 Improvements in Composite Steel Plates, &c., of which the following is a specification.

The object of my invention is to prepare slabs or plates having a hard resisting surface, and a softer and more yielding backing, 10 an object which I attain in the manner hereinafter set forth, reference being had to the accompanying drawings, in which the three figures represent successive stages in the preparation of a plate in accordance with my 15 invention.

Figure 1 is a sectional view of the plate at the end of the first stage; Fig. 2, a similar view at the end of the second stage, and Fig. 20 3, a similar view at the end at the third and last stage.

In carrying out my invention I first produce, by casting or otherwise, a soft steel plate and then, while the same is highly heated, cast upon the face of the same a layer 25 of iron, which is afterward subjected to any of the usual processes whereby partial decarbonization of the same is effected for the purpose of converting it into steel capable of being hardened and tempered, and is finally tempered throughout the whole or a part of its mass. By this means I am enabled to produce 30 a plate having a surface of any desired degree of hardness and a back of softer metal the two being firmly united, for it has been found in practice that by casting the mass of iron upon the face of a body of highly heated steel, an 35 intimate union of the two bodies is effected and a homogeneous block or plate is produced.

In carrying out my invention a body of steel 40 A may be first run into the bottom of a mold, and the body of cast iron B may then be poured in directly upon the top of this mass of steel, the greater specific gravity of the latter being relied upon to prevent the disturbance of the 45 same by the pouring of the iron on top of it, although it will be preferable to permit the steel to partially cool before pouring the iron into the mold, the steel, however, still retaining a high degree of heat when the iron is 50 brought into contact with it, or a steel plate, slab or block produced in any available manner may be first highly heated and then in-

duced into the mold in order to provide a base upon which to pour the mass of cast iron. When the composite block such as shown in 55 Fig. 1 has become cold, or sufficiently cool to permit handling, the cast iron portion of the block is subjected to any of the ordinary converting operations whereby partial decarbonization of the iron can be effected and the same 60 reduced to a condition for being hardened and tempered, the composite plate at this stage being represented in Fig. 2, where the converted portion of the plate is represented at B'. For carrying out this part of the process I may resort to the treatment set forth in my Patent 65 No. 498,062, dated May 23, 1893, or the iron portion of the composite plate may be subjected to any of the usual cementation processes and may be afterward hardened or tempered 70 in any ordinary manner throughout either the whole or a part of its mass, as shown in Fig. 3, where the hardened or tempered portion of the plate is represented at B<sup>2</sup>, the mass of steel forming the backing for the mass 75 of iron being protected from injury or change during such converting, hardening and tempering operations, so that it preserves its original character and provides a backing for the hardened or tempered face of the plate. 80

My invention is of special advantage in the manufacture of armor plates or armor piercing projectiles, the latter having an outer surface of hardened steel and an interior core or heart of soft steel. 85

Having thus described my invention, I claim and desire to secure by Letters Patent—

The mode herein described of producing plates, blocks, or other articles having a hardened steel face, with a soft steel backing, said mode consisting in casting a mass of iron upon a backing of steel, converting said cast iron mass into steel capable of being hardened or tempered, and then hardening or tempering the same, substantially as specified. 90 95

In testimony whereof I have signed my name to this specification in the presence of two subscribing witnesses.

JNO. A. HUNTER.

Witnesses:

WILLIAM A. BARR,  
JOSEPH H. KLEIN.